

# United States Patent [19]

Sharmaitis et al.

[11] 3,855,010

[45] Dec. 17, 1974

[54] COMPOSITION AND METHOD FOR COLOR PASSIVATION OF ZINC AND CADMIUM

[76] Inventors: **Romas Romovich Sharmaitis**, ulitsa Antakalne, 93, kv. 24; **Valentina Alexeevna Vilutene**, ulitsa Zhvaigzhdju 4, kv. 243; **Juozas Juozovich Matulis**, ulitsa Malonei 11, kv. 1, all of Vilnjus, U.S.S.R.

[22] Filed: Dec. 29, 1972

[21] Appl. No.: 319,391

[30] Foreign Application Priority Data

Apr. 5, 1972 U.S.S.R. .... 1762901

[52] U.S. Cl. .... 148/6.21, 148/6.2

[51] Int. Cl. .... C23f 7/26

[58] Field of Search .... 148/6.21, 6.2

[56] References Cited

UNITED STATES PATENTS

|           |         |                  |          |
|-----------|---------|------------------|----------|
| 2,904,414 | 9/1959  | Ostrander et al. | 148/6.21 |
| 3,121,032 | 2/1964  | Seyb             | 148/6.21 |
| 2,483,510 | 10/1949 | Stareck          | 148/6.21 |

|           |        |               |          |
|-----------|--------|---------------|----------|
| 3,307,980 | 3/1967 | Freeman       | 148/6.21 |
| 3,519,501 | 7/1970 | Holden et al. | 148/6.2  |

Primary Examiner—Ralph S. Kendall  
Attorney, Agent, or Firm—Holman & Stern

[57] ABSTRACT

A composition comprising a mixture of hexavalent chromium compounds such as chromic anhydride and soluble chromates, and soluble nitrates, soluble sulphates, soluble boron compounds, and an amino acid, said composition having the following content of the above components (in weight parts):

|                                                          |          |
|----------------------------------------------------------|----------|
| hexavalent chromium compound<br>(calculated as chromium) | 1.7-70.0 |
| nitrate compound (calculated as $\text{NO}_3^-$ )        | 1.0-45.0 |
| sulphate compound (calculated as $\text{SO}_4^{2-}$ )    | 1.0-25.0 |
| boron compound (calculated as boron)                     | 0.5-10.0 |
| amino acid                                               | 0.5-6.0  |

Passivation is effected by dipping the workpieces into an aqueous solution of said composition for a period of 3 to 90 seconds at a temperature of 15° to 35°C.

12 Claims, No Drawings

# COMPOSITION AND METHOD FOR COLOR PASSIVATION OF ZINC AND CADMIUM

The present invention relates to improvements in compositions and methods for the chemical treatment of metal surfaces, and more particularly to a composition and a method for color passivation of zinc and cadmium. The invention is of particular advantage in providing a color passive film on zinc and cadmium in order to increase the corrosion resistance of articles made therefrom, or articles having a zinc or cadmium surface, such as zinc- or cadmium-based alloys, zinc castings, and, specifically, articles having a zinc- or cadmium-plated coating.

Zinc and cadmium become corroded in a relatively short time under the effect of atmospheric moisture. In order to extend the life of articles having a zinc or cadmium surface and to preserve their decorative appearance, they may be passivated in acid solutions of hexavalent chromium. Aqueous solutions are known in this art for passivating zinc and cadmium containing chromic anhydride, sulphate ions, boric and nitric acids (cf. U.S. Pat. No. 2,904,414), or hexavalent chromium, sulphate ions, nitrate ions and acetate or borate ions (cf. U.S. Pat. No. 3,121,032).

The use of a solution containing chromic anhydride, sulphate ions, boric and nitric acids involves intensive dissolving of the metal being passivated, particularly when an automatic passivating apparatus is employed. The preparation of the passivating solution and the process of passivating proper requires great amounts of concentrated nitric acid which presents difficulties in properly controlling the composition of the solution because of rapid accumulation of foreign matter therein. A zinc or cadmium surface passivated in such a solution does gain a decorative appearance, while its corrosion resistance increases only slightly.

The solution containing hexavalent chromium, sulphate ions, nitrate ions, and acetate or borate ions is conductive to the formation of colorless passive films on articles having a zinc or cadmium surface, but again their corrosion resistance fails to increase significantly.

The above methods can be applied in order to obtain decorative films on articles having a zinc or cadmium surface. However, when tested in a fog of a neutral 5% aqueous solution of sodium chloride, a zinc or cadmium surface shows its first signs of corrosion even before a 20 to 30 hour period has expired.

It is an object of the present invention to provide a dry composition for preparing a solution for color passivation, in manual, or automatic apparatus.

Another object of the invention is to provide a dry composition for adjusting the solution for color passivation of zinc and cadmium.

Still another object of the invention is to provide a solution for color passivation of zinc and cadmium which does not require frequent replacement, but which is makes it possible to replenish or make adjustment during the course of passivating.

Yet another object of the invention is to provide a method for obtaining color passive films on zinc and cadmium possessing high corrosion resistance.

These and other objects are achieved by applying a novel composition which is, according to the invention, a mixture of hexavalent chromium compounds, such as chromic anhydride and/or soluble chromates, and soluble nitrate compounds, soluble sulphate compounds,

soluble boron compounds and, an amino acid of the general formula:



10 where  $\text{R}_1, \text{R}_2, \text{R}_3, \text{R}_4 = -\text{H}$ , alkyl ( $\text{C}_1-\text{C}_8$ ), phenyl, substituents and phenyls, containing substituents  $-\text{OH}$ ,  $\text{R}_1-\text{OR}$ ,  $-\text{COR}$ ,  $-\text{COOH}$ ,  $-\text{COOR}$ ,  $-\text{CONH}_2$ ,  $-\text{CN}_1$ ,  $-\text{NH}_2$ ,  $-\text{NHR}$ ,  $\text{RNR}$  ( $\text{R} = \text{alkyl}$  and aryl),  $n = 1 - 5$ , with said composition having the following content of the above components (in weight parts).

|                                                          |          |
|----------------------------------------------------------|----------|
| hexavalent chromium compound<br>(calculated as chromium) | 1.7-70.0 |
| nitrate compound (calculated as $\text{NO}_3^-$ )        | 1.0-45.0 |
| sulphate compound (calculated as $\text{SO}_4^{2-}$ )    | 1.0-25.0 |
| boron compound (calculated as boron)                     | 0.5-10.0 |
| amino acid                                               | 0.05-6.0 |

25 Hexavalent chromium compounds constitute the basic passivating agent. Its content in a composition for color passivation of zinc and cadmium should be 1.7 to 70.0 weight parts. Sulphate compounds are the main activators of the passivating process. Their concentration in a passivating composition, when calculated as  $\text{SO}_4^{2-}$ , should vary from 1.0 to 25.0 weight parts. Nitrate compounds act as the oxidizing and brightening agents. Their concentration in the passivating composition, when calculated as  $\text{NO}_3^-$ , should be maintained within 1.0 to 45.0 weight parts. Boron compounds impart the polishing and brightening properties to the composition. Their concentration in a composition, when calculated as boron, should be from 0.5 to 10.0 weight parts. Amino acids are the stabilizing and buffering agents ensuring an extremely long life for the passivating composition. Their content in a composition should be from 0.05 to 6.0 weight parts.

30 It is expedient that a passivating composition contain (in weight parts):

|                                                          |           |
|----------------------------------------------------------|-----------|
| hexavalent chromium compound<br>(calculated as chromium) | 11.0-21.0 |
| nitrate compound (calculated as $\text{NO}_3^-$ )        | 2.4-6.0   |
| sulphate compound (calculated as $\text{SO}_4^{2-}$ )    | 2.2-7.0   |
| boron compound (calculated as boron)                     | 1.1-4.3   |
| amino acid                                               | 0.05-0.1  |

45 50 The stabilizing and buffering action of the amino acids becomes manifest even at a low concentration thereof in a passivating solution. That is why, in order to prepare and replenish a passivating solution in an apparatus where substantial losses of the solution are suffered through an intensive carrying away thereof by the workpiece surface, it would be most advantageous to use the above composition wherein the amino acid content is from 0.05 to 0.1 weight parts.

55 It is most expedient that a passivating composition contain (in weight parts):

|                                                          |           |
|----------------------------------------------------------|-----------|
| hexavalent chromium compound<br>(calculated as chromium) | 11.0-21.0 |
| nitrate compound (calculated as $\text{NO}_3^-$ )        | 2.4-6.0   |
| sulphate compound (calculated as $\text{SO}_4^{2-}$ )    | 2.2-7.0   |
| boron compound (calculated as boron)                     | 1.1-4.3   |
| amino acid                                               | 0.5-4.0   |

It is advisable that the hexavalent chromium be introduced into the composition as chromic anhydride compounds; chromates of ammonium, beryllium, potassium, cadmium, lithium, magnesium, sodium, zinc; bichromates of ammonium, beryllium, potassium, cadmium, lithium, magnesium, sodium, zinc; mixtures of said chromates; mixtures of said bichromates; mixtures of chromic anhydride and chromates; mixtures of chromic anhydride and bichromates; and mixtures of chromic anhydride, chromates and bichromates, all being taken separately or in combinations.

It is most advisable that the nitrate be introduced into the composition as nitrate compounds of ammonium, beryllium, potassium, sodium, cadmium, lithium, magnesium, zinc, all being taken separately or in combinations.

It is also advisable that the sulphate be introduced into the composition as sulphate compounds of ammonium, beryllium, potassium, cadmium, lithium, magnesium, sodium, zinc, bisulphate compounds of ammonium, potassium, lithium, and sodium, all being taken separately or in combinations.

The boron should be preferably introduced into the composition as the following compounds: boric acid, magnesium orthoborate, and polyborates of ammonium, beryllium, potassium, lithium, magnesium, sodium, all being taken separately or in combinations.

It is most expedient that the amino acid have the general formula:



where  $\text{R}_1$  and  $\text{R}_2$  stand for  $-\text{H}$ ,  $-\text{CH}_3$ ,  $-\text{C}_2\text{H}_5$ ,  $-\text{C}_3\text{H}_7$ ,  $-\text{C}_4\text{H}_9$ ,  $-\text{C}_6\text{H}_5$ ,  $-\text{CH}_2\text{OOH}$ ,  $-\text{CH}_2\text{CH}_2\text{COOH}$ ,  $-\text{CH}_2\text{CH}_2\text{OH}$ ,  $-\text{CH}_2\text{CH}_2\text{CN}$ ,  $\text{CH}_2\text{CH}_2\text{COCH}_2$ ,  $-\text{CH}_2\text{CH}_2\text{COC}_2\text{H}_5$ ,  $-\text{CH}_2\text{CH}_2\text{COC}_3\text{H}_7$ ,  $-\text{CH}_2\text{CH}_2\text{COC}_6\text{H}_5$ ,  $\text{R}_3$  and  $\text{R}_4$ , for  $-\text{H}$ ,  $-\text{CH}_3$ ,  $-\text{C}_2\text{H}_5$ ,  $-\text{C}_3\text{H}_7$ ,  $-\text{C}_4\text{H}_9$ ,  $-\text{C}_5\text{H}_{11}$ ,  $-\text{C}_6\text{H}_{13}$ ,  $-\text{C}_7\text{H}_{15}$ ,  $-\text{C}_8\text{H}_{17}$ ,  $-\text{CH}_2\text{COOH}$ ,  $-\text{CH}_2\text{CH}_2\text{COOH}$ ,  $-(\text{CH}_2)_k\text{NH}_2$ ,  $-(\text{CH}_2)_k$



$\text{C}_6\text{H}_5$ ,

maybe  $\text{K}=1-4$ ; and  $n=1-5$

The invention, according to one embodiment thereof, can provide a composition having the following content of its ingredients in an aqueous solution thereof (in g/l):

|                                                          |          |
|----------------------------------------------------------|----------|
| hexavalent chromium compound<br>(calculated as chromium) | 1.7-70.0 |
| nitrate compound (calculated as $\text{NO}_3^-$ )        | 1.0-45.0 |
| sulphate compound (calculated as $\text{SO}_4^{2-}$ )    | 1.0-25.0 |
| boron compound (calculated as boron)                     | 0.5-10.0 |
| amino acid                                               | 0.05-6.0 |
| solution pH = 1.1 - 2.8                                  |          |

It is expedient that the content of the composition ingredients in an aqueous solution thereof be (in g/l):

hexavalent chromium compound

-Continued

|   |                                                       |           |
|---|-------------------------------------------------------|-----------|
| 5 | (calculated as chromium)                              | 11.0-21.0 |
|   | nitrate compound (calculated as $\text{NO}_3^-$ )     | 2.4-6.0   |
|   | sulphate compound (calculated as $\text{SO}_4^{2-}$ ) | 2.2-7.0   |
|   | boron compound (calculated as boron)                  | 1.1-4.3   |
|   | amino acid                                            | 0.05-1.1  |
|   | solution pH = 1.6-2.3                                 |           |

It is most expedient that the content of the composition ingredients in the aqueous solution thereof be (in g/l):

|    |                                                          |           |
|----|----------------------------------------------------------|-----------|
| 10 | hexavalent chromium compound<br>(calculated as chromium) | 11.0-21.0 |
|    | nitrate compound (calculated as $\text{NO}_3^-$ )        | 2.4-6.0   |
|    | sulphate compound (calculated as $\text{SO}_4^{2-}$ )    | 2.2-7.0   |
|    | boron compound (calculated as boron)                     | 1.1-4.3   |
|    | amino acid                                               | 0.5-4.0   |

20 The novel method for passivating zinc and cadmium by dipping them into an aqueous solution containing a hexavalent chromium compound comprises using a composition having the following ingredient contents in an aqueous solution thereof (in g/l):

|    |                                                          |          |
|----|----------------------------------------------------------|----------|
| 25 | hexavalent chromium compound<br>(calculated as chromium) | 1.7-70.0 |
|    | nitrate compound (calculated as $\text{NO}_3^-$ )        | 1.0-45.0 |
|    | sulphate compound (calculated as $\text{SO}_4^{2-}$ )    | 1.0-25.0 |
|    | boron compound (calculated as boron)                     | 0.5-10.0 |
|    | amino acid                                               | 0.05-6.0 |

30 35 the pH of the solution is from 1.1 to 2.8, and the zinc or cadmium is treated therein at a temperature of from 15° to 35°C for a period of about 3 to 90 seconds.

30 The proposed composition for color passivating zinc and cadmium is a mixture of non-volatile solid substances which is easy to prepare, to transport, to store and to use. The latter requirement is attained by an easy preparation of the passivating solution, as well as in the facile adjustment and control thereof. If necessary, the composition may be prepared on the spot by conventional mechanical blending starting ingredients.

40 45 After the treatment by the proposed method, a bright color passive film is formed on the zinc or cadmium surface. This passive film has bright opalescent tints even if the zinc or cadmium surface was dull prior to treatment.

50 55 The passive films obtained by the novel method are abrasion-resistant in the course of passivating, therefore use may be made of manually operated and automatic apparatus of both stationary and rotary type may be used.

60 One of the chief advantages of the present invention is that the passive films obtained by the method provided herein have a high corrosion resistance. The passive film formed on a zinc or cadmium surface is tested for corrosion resistance by the so-called "salt fog" method whereby the film is subjected to a continuous action of a fog produced by spraying in a testing cabinet with a 5% aqueous neutral solution of sodium chloride at a temperature of 35° ± 1°C. The corrosion resistance of a film is determined by the time interval between the onset of the test and the moment of the ap-

pearance of the first signs of corrosion on the film surface.

The first signs of corrosion of zinc and cadmium after passivation by the herein disclosed novel method appear only after 90 to 100 hours.

Other objects and advantages of the invention will become more apparent from the following detailed description of specific embodiments thereof.

Given below in Examples 1 to 6 are the various amounts for preparing and adjusting a solution for color passivation of zinc or cadmium. The contents are given in weight parts.

|                                                        |      |
|--------------------------------------------------------|------|
| Example 1.                                             |      |
| chromic anhydride (calculated as chromium)             | 10.0 |
| potassium chromate (calculated as chromium)            | 5.0  |
| cadmium nitrate (calculated as $\text{NO}_3^-$ )       | 5.2  |
| potassium sulphate (calculated as $\text{SO}_4^{2-}$ ) | 4.3  |
| sodium tetraborate (calculated as boron)               | 2.0  |
| $\alpha$ -amino glutaric acid                          | 1.75 |
| Example 2.                                             |      |
| sodium bichromate (calculated as chromium)             | 18.3 |
| potassium nitrate (calculated as $\text{NO}_3^-$ )     | 3.2  |
| beryllium sulphate (calculated as $\text{SO}_4^{2-}$ ) | 1.2  |
| boric acid (calculated as boron)                       | 2.7  |
| $\alpha$ -amino glutaric acid                          | 0.08 |
| Example 3.                                             |      |
| chromic anhydride (calculated as chromium)             | 70.0 |
| ammonium nitrate (calculated as $\text{NO}_3^-$ )      | 20.1 |
| lithium sulphate (calculated as $\text{SO}_4^{2-}$ )   | 25.0 |
| magnesium orthoborate (calculated as boron)            | 0.5  |
| N-(p-ethoxyphenyl)- $\beta$ -aminopropionic acid       | 3.3  |
| Example 4.                                             |      |
| beryllium bichromate (calculated as chromium)          | 5.6  |
| lithium chromate (calculated as chromium)              | 7.4  |
| zinc nitrate (calculated as $\text{NO}_3^-$ )          | 1.0  |
| cadmium sulphate (calculated as $\text{SO}_4^{2-}$ )   | 1.9  |
| ammonium pentaborate (calculated as boron)             | 10.0 |
| N-octylamino-acetic acid                               | 6.0  |
| Example 5.                                             |      |
| zinc bichromate (calculated as chromium)               | 26.3 |
| magnesium bichromate (calculated as chromium)          | 13.6 |
| lithium nitrate (calculated as $\text{NO}_3^-$ )       | 45.0 |
| sodium bisulphite (calculated as $\text{SO}_4^{2-}$ )  | 18.3 |
| zinc borate (calculated as boron)                      | 2.6  |
| $\alpha$ ( $\beta$ -cyanoethyl)-amino-acetic acid      | 0.8  |
| Example 6.                                             |      |
| chromic anhydride (calculated as chromium)             | 1.7  |
| magnesium nitrate (calculated as $\text{NO}_3^-$ )     | 4.3  |
| beryllium sulphate (calculated as $\text{SO}_4^{2-}$ ) | 4.3  |
| boric acid (calculated as boron)                       | 1.0  |
| N-(B-hydroxyethyl)-imino-di-acetic acid                | 0.05 |

Illustrative examples of other amino acids used in the above compositions are:

1. Nitrilotriacetic acid
2. Imino-di-acetic acid
3. N-phenyl-imino-di-acetic acid
4. Amino-acetic acid

-Continued

|     |                                                              |
|-----|--------------------------------------------------------------|
| 5.  | N,N-dimethyl-amino-acetic acid                               |
| 6.  | N,N-diethyl-amino-acetic acid                                |
| 7.  | N,N-di(B-hydroxyethyl)-amino-acetic acid                     |
| 8.  | N-( $\beta$ -aminoethyl)-amino-acetic acid                   |
| 9.  | $\alpha$ -aminopropionic acid                                |
| 10. | N-( $\beta$ -cyanoethyl)- $\alpha$ -aminopropionic acid      |
| 11. | $\alpha$ ( $\beta$ -cyanoethyl)-amino-acetic acid            |
| 12. | N-( $\beta$ -benzoylethyl)- $\alpha$ -amino butyric acid     |
| 13. | $\beta$ -aminopropionic acid                                 |
| 14. | $\beta$ -amino isobutyric acid                               |
| 15. | $\beta$ -dimethyl-amino- $\beta$ -phenyl-propionic acid      |
| 16. | $\beta$ -dimethylamino-butyric acid                          |
| 17. | N,N-di( $\beta$ -carboethoxyethyl)-amino-acetic acid         |
| 18. | N-(n-dimethyl-aminophenyl)- $\alpha$ -aminopropionic acid    |
| 19. | $\gamma$ -aminobutyric acid                                  |
| 20. | $\epsilon$ -aminocaproic acid                                |
| 21. | N-carboxymethyl- $\alpha$ -aminopropionic acid               |
| 22. | $\alpha$ (carboxymethyl-amino)- $\beta$ -aminopropionic acid |
| 23. | Aminosuccinic acid                                           |
| 24. | $\alpha$ -amino butyric acid                                 |
| 25. | $\alpha$ -aminoisobutyric acid                               |
| 26. | $\alpha$ -amino- $\beta$ -carbamido-propionic acid           |
| 27. | $\alpha$ -aminoisovaleric acid                               |
| 28. | $\alpha$ -aminocaproic acid                                  |
| 29. | $\alpha$ -aminoisocaproic acid                               |
| 30. | $\alpha$ -amino- $\beta$ -phenyl-propionic acid.             |

A passivating solution is prepared by dissolving the dry passivating composition in water. In practical use, 25 the solution is, if necessary, adjusted with an acid such as sulphuric acid, or a hydroxide such as sodium hydroxide, to maintain the solution pH within a range of from 1.1 to 2.8. The preferable pH of the passivating solution within this range depends on the time of the 30 treatment of a zinc or cadmium surface by the solution. In case the passivation takes little time (3 to 8 seconds), the optimum pH would be 1.1 to 1.7, and if passivating treatment lasts longer (20 to 16 seconds), the optimum pH would be from 1.7 to 2.5. For in order to 35 obtain color passive films, on articles having a zinc or cadmium surface, said color passive films having a high corrosion resistance, as well as resistant to wet attrition, by using a passivating solution on a rotary apparatus, the optimum pH of the solution would be from 1.6 to 40 2.3.

When said solutions are used for color passivation of zinc and cadmium, their temperature should be maintained within a range of from 15° to 35°C and, in order 45 to obtain the best results, within a range of from 20° to 28°C.

The time for treatment of a zinc or cadmium surface with a passivating solution may vary from 3 to 90 sec, 50 but usually it lies within 10 to 35 seconds. The higher the pH, the lower are the temperature and the concentration of the ingredients of the solution and the longer the time of passivation, and vice versa.

According to the present invention, articles having a zinc or cadmium surface are dipped into a passivating solution for a definite period of time depending on the properties of the solution, then removed therefrom, rinsed in running cold water, then in heated water, and, 60 finally, dried. As a result of such treatment, the zinc or cadmium surface is coated with a color opalescent passive film of high corrosion resistance.

Given in Table 1 are the tolerable and optimum concentrations of ingredients of solutions for color passivation of zinc and cadmium according to the present invention.

| Ingredient                                            | Permissible concentration (g/l) | Optimum concentration (g/l) | Optimum concentration (g/l) |
|-------------------------------------------------------|---------------------------------|-----------------------------|-----------------------------|
| Hexavalent chromium compound (calculated as chromium) | 1.7-70.0                        | 11.0-21.0                   | 11.0-21.0                   |
| Nitrate compound (calculated as $\text{NO}_3^-$ )     | 1.0-45.0                        | 2.4-6.0                     | 2.4-6.0                     |
| Sulphate compound (calculated as $\text{SO}_4^{2-}$ ) | 1.0-25.0                        | 2.2-7.0                     | 2.2-7.0                     |
| Boron compound (calculated as boron)                  | 0.5-10.0                        | 1.1-4.3                     | 1.1-4.3                     |
| Amino acid                                            | 0.05-6.0                        | 0.05-0.1                    | 0.5-4.0                     |

In case a passivating solution is used on an apparatus noted for substantial losses thereof through being carried away by the workpiece surface, it is more preferable that the solution contain less amino acid.

In the course of passivation, the concentration of the solution ingredients is constantly diminishing due to a reaction between the workpiece surface and the solution, and a dilution of the solution. An outstanding feature of the present invention is the possibility of replenishing and adjusting the passivating solution, in the course of passivating the treatment, by adding the above dry passivating compositions and an acid in the amounts is dictated by the assays, e.g. hexavalent chromium and pH.

The novel method for color passivation of zinc and cadmium according to the invention is illustrated by Examples 7 and 8.

#### EXAMPLE 7.

208.74 g of the dry composition of Example 1 were dissolved in 3 of water. After adding 1.0 ml/l of  $\text{H}_2\text{SO}_4$  ( $d = 1.83$ ) to a pH of 1.86, a passivating solution was obtained containing (in g/l):

|                        |      |
|------------------------|------|
| hexavalent chromium    | 15.1 |
| $\text{NO}_3^-$ ion    | 5.2  |
| $\text{SO}_4^{2-}$ ion | 6.1  |
| boron                  | 2.0  |
| amino acid             | 1.75 |

A steel workpiece was immersed into the prepared solution maintained at 23°C was and, coated with bright zinc in a cyanide bath for zinc-plating, for a period of 20 sec. At the expiration of this period, the workpiece was taken out, rinsed in running cold water and then in heated (to 40°C) water, and dried in hot (60°C) air. As a result of this treatment, the zinc surface was coated with a bright color film with opalescent tints.

Said solution was further used for passivating zinc articles. In the course of passivating, the solution was replenished with sulphuric acid and the dry passivating composition of Example 1 in amounts as based on the assays for pH and hexavalent chromium. Throughout the passivating process, the solution was adjusted by adding an amount of dry composition sufficient for the volume of the solution to become five-fold of that of which it originally was. After passivating zinc plated surfaces of 0.1, 1.0, 10.0 and 30.0 square meters the, samples were taken for corrosion tests in a salt-fog cab-

inet. The first signs of corrosion appeared, in the first three cases, after 120 hours and, in the fourth case, after 100 hours of testing.

#### EXAMPLE 8.

750.0 g of the dry composition of Example 2 were dissolved in a 10 l-capacity bath on a rotary automatic apparatus noted for its marked dilution and for carrying away the passivating solution due to a large surface of the work being passivated. After adding 0.55 ml/l of sulphuric acid ( $d = 1.83$ ) to a pH of 2.16, a passivating solution was obtained containing (in g/l):

|                        |      |
|------------------------|------|
| hexavalent chromium    | 18.3 |
| $\text{NO}_3^-$ ion    | 3.2  |
| $\text{SO}_4^{2-}$ ion | 2.2  |
| boron                  | 2.7  |
| amino acid             | 0.08 |

Immersed into the prepared solution maintained at 25°C for a period of 30 seconds was a drum loaded with steel workpieces coated with matte cadmium in a cyanide bath for cadmium-plating. At the expiration of this period, the drum was taken out, dipped into a bath with running cold water for a period of 30 seconds, then into a bath of heated (to 40°C) water for a period of 30 seconds, and, finally, transferred to a desiccator where the cadmium-plated work-pieces were dried after passivation in hot (60°C) air. As a result of this treatment, the cadmium-plated workpieces were coated with a bright color film with opalescent tints.

The passivation of the cadmium-plated workpieces continued in said apparatus. In the course of passivation, the solution was replenished with sulphuric acid and the dry passivating composition of Example 2 in amounts as based on the assay for pH and hexavalent chromium. Throughout the passivating process, the solution was adjusted by adding an amount of dry composition sufficient to attain a twenty-fold increase of the initial solution volume. After passivating 0.4, 4.0, 40 and 120 square meters of the cadmiumplated surface, the samples were taken for corrosion tests in a salt-fog cabinet. The first signs of corrosion appeared, in the first three cases, after 148 hours and, in the fourth case, after 120 hours of testing.

#### EXAMPLES 9 to 21.

Shown in table 2 various compositions of passivating solutions and the conditions for passivating zinc and cadmium therein.

Table 2

| Example No.                   | : 9  | : 10 | : 11 | : 12 | : 13 | : 14 | : 15 | : 16 | : 17 | : 18 | : 19 | : 20 | : 21 |
|-------------------------------|------|------|------|------|------|------|------|------|------|------|------|------|------|
| <b>INGREDIENTS</b>            |      |      |      |      |      |      |      |      |      |      |      |      |      |
| (in g/l)                      |      |      |      |      |      |      |      |      |      |      |      |      |      |
| Cr (VI)                       | 32.2 | 11.6 | 13.0 | 70.0 | 5.5  | 10.2 | 1.7  | 5.0  | 9.0  | 4.8  | 20.3 | 11.4 | 5.38 |
| NO <sub>3</sub> <sup>-</sup>  | 18.6 | 2.3  | 1.0  | 20.1 | 5.0  | 1.0  | 4.3  | 3.6  | 1.0  | 1.3  | 1.0  | 4.81 | 10.6 |
| SO <sub>4</sub> <sup>2-</sup> | 4.3  | 3.6  | 4.6  | 25.0 | 2.7  | 2.8  | 1.0  | 4.4  | 5.2  | 1.2  | 1.07 | 7.08 | 6.8  |
| B                             | 2.2  | 0.94 | 10.0 | 0.5  | 0.5  | 1.9  | 3.0  | 0.5  | 1.08 | 0.5  | 0.57 | 1.13 | 2.98 |
| amino acid                    | 4.2  | 2.7  | 6.0  | 3.3  | 0.93 | 0.5  | 0.05 | 2.0  | 0.26 | 0.48 | 3.44 | 1.0  | 2.04 |
| pH                            | 1.35 | 2.06 | 2.8  | 1.1  | 1.25 | 1.62 | 2.45 | 1.35 | 1.8  | 1.33 | 1.89 | 1.52 | 1.6  |
| t°C                           | 20   | 27   | 15   | 22   | 27   | 20   | 35   | 22   | 25   | 20   | 25   | 20   | 30   |
| t, sec                        | 20   | 60   | 90   | 3    | 10   | 40   | 30   | 35   | 30   | 15   | 25   | 20   | 40   |

**EXAMPLE 9.**

A passivating solution was prepared by dissolving in water the respective amounts of chromic anhydride, sodium nitrate, zinc sulphate, lithium tetraborate, and N-( $\beta$ -benzoylethyl)- $\alpha$ -amino butyric acid.

**EXAMPLE 10.**

A passivating solution was prepared by dissolving in water the respective amounts of sodium bichromate, cadmium nitrate, potassium sulphate, sodium tetraborate, and  $\alpha$ -aminocaproic acid.

**EXAMPLE 11.**

A passivating solution was prepared by dissolving in water the composition of Example 4.

**EXAMPLE 12.**

A passivating solution was prepared by dissolving in water the composition of Example 3.

**EXAMPLE 13.**

A passivating solution was prepared by dissolving in water the respective amounts of potassium chromate, beryllium nitrate, zinc sulphate, boric acid, and  $\alpha$ -amino- $\beta$ (phenyl)-propionic acid.

**EXAMPLE 14.**

A passivating solution was prepared by dissolving in water the respective amounts of ammonium bichromate, potassium nitrate, potassium sulphate, lithium tetraborate, and  $\alpha$ -amino-isocaproic acid.

**EXAMPLE 15.**

A passivating solution was prepared by dissolving in water the composition of Example 6.

**EXAMPLE 16.**

A passivating solution was prepared by dissolving in water the respective amounts of sodium chromate, sodium nitrate, sodium sulphate, potassium tetraborate, and  $\beta$ -aminopropionic acid.

**EXAMPLE 17.**

A passivating solution was prepared by dissolving in water the respective amounts of potassium bichromate, beryllium sulphate, zinc nitrate, potassium pentaborate, and  $\alpha$ -amino-succinic acid.

**EXAMPLE 18.**

A passivating solution was prepared by dissolving in water the respective amounts of chromic anhydride,

sodium chromate, magnesium nitrate, cadmium sulphate, sodium tetraborate, and  $\alpha$ ( $\beta$ '-cyanoethyl)-15 amino-acetic acid.

**EXAMPLE 19.**

A passivating solution was prepared by dissolving in water the respective amounts of chromic anhydride, potassium chromate, zinc nitrate, lithium sulphate, zinc borate, and  $\alpha$ -aminoisovaleric acid.

**EXAMPLE 20.**

A passivating solution was prepared by dissolving in water the respective amounts of chromic anhydride, lithium sulphate, potassium nitrate, sodium tetraborate, and  $\alpha$ -aminopropionic acid.

**EXAMPLE 21.**

A passivating solution was prepared by dissolving in water the respective amounts of chromic anhydride, sodium chromate, beryllium nitrate, potassium sulphate, lithium tetraborate, and N,N-diethyl-aminoacetic acid.

In Examples 9, 12, 15, 19 and 20, the solution was adjusted in order to obtain the pH value given in Table 2 by adding therein sodium hydroxide, while in the other Examples, sulphuric acid was added for the same purpose.

Steel workpieces were passivated in Examples 10, 11, 15, 18 and 20 having a bright zinc coating obtained in a cyanide bath, in Example 16, steel workpieces with a matte zinc coating obtained in a cyanide bath were passivated, and in Examples 9, 13 and 19, steel workpieces with a bright cadmium coating obtained in a cyanide bath, in Example 21, steel workpieces with a matte cadmium coating obtained in a cyanide bath, in Example 12, workpieces made of a zinc alloy, in Example 14, workpieces made of a zinc casting, and in Example 17, a steel workpiece coated with zinc by a hot process were also passivated.

In Examples 14, 15 and 20, passivation was effected by following the procedure of Example 8, and in the other Examples, the workpieces were passivated by following the procedure of Example 7.

In each case, the treated workpieces were coated with a color opalescent film. The brightest films were obtained in Examples 9, 10, 13, 18 and 20.

The corrosion resistance of the passive films obtained by the novel method and which were tested in a "salt fog" cabinet is given in Table 3.

Table 3

| Example No.                                                                                            | 9   | 10  | 11 | 12  | 13  | 14 | 15 | 16  | 17  | 18  | 19  | 20 | 21  |
|--------------------------------------------------------------------------------------------------------|-----|-----|----|-----|-----|----|----|-----|-----|-----|-----|----|-----|
| Time period between the onset of the test and the appearance of the first signs of corrosion, in hours | 130 | 120 | 96 | 106 | 108 | 96 | 90 | 114 | 102 | 108 | 120 | 96 | 124 |

What is claimed is:

1. A composition for the color passivation of zinc and cadmium consisting essentially of a mixture of hexavalent chromium compounds selected from the group consisting of chromic anhydride and soluble chromates, and soluble nitrate compounds, soluble sulphate compounds, soluble boron compounds, and an amino acid of the general formula:



where  $R_1, R_2, R_3, R_4 = -H$ , alkyl ( $C_1-C_8$ ), phenyl, substituted alkyls and phenyls, containing substituents  $-\text{OH}$ ,  $-\text{R}$ ,  $-\text{COR}$ ,  $-\text{COOH}$ ,  $-\text{COOR}$ ,  $-\text{CONH}_2$ ,  $-\text{CN}_1$ ,  $-\text{NH}_2$ ,  $-\text{NHR}$ ,  $-\text{RNR}$ , ( $\text{R} = \text{alkyl, and aryl}$ ),  $n = 1 - 5$ , said composition having the following content of the above components (in weight parts):

|                                                       |          |
|-------------------------------------------------------|----------|
| hexavalent chromium compound (calculated as chromium) | 1.7-70.0 |
| nitrate compound (calculated as $\text{NO}_3^-$ )     | 1.0-45.0 |
| sulphate compound (calculated as $\text{SO}_4^{2-}$ ) | 1.0-25.0 |
| boron compound (calculated as boron)                  | 0.5-10.0 |
| amino acid                                            | 0.05-6.0 |

2. A composition for color passivation of zinc and cadmium as claimed in claim 1, containing (in weight parts):

|                                                       |           |
|-------------------------------------------------------|-----------|
| hexavalent chromium compound (calculated as chromium) | 11.0-21.0 |
| nitrate compound (calculated as $\text{NO}_3^-$ )     | 2.4-6.0   |
| sulphate compound (calculated as $\text{SO}_4^{2-}$ ) | 2.2-7.0   |
| boron compound (calculated as boron)                  | 1.1-4.3   |
| amino acid                                            | 0.05-0.1  |

3. A composition for color passivation of zinc and cadmium as claimed in claim 1, containing (in weight parts):

|                                                       |           |
|-------------------------------------------------------|-----------|
| hexavalent chromium compound (calculated as chromium) | 11.0-21.0 |
| nitrate compound (calculated as $\text{NO}_3^-$ )     | 2.4-6.0   |
| sulphate compound (calculated as $\text{SO}_4^{2-}$ ) | 2.2-7.0   |
| boron compound (calculated as boron)                  | 1.1-4.3   |
| amino acid                                            | 0.5-4.0   |

4. A composition for the color passivation of zinc and cadmium as claimed in claim 1, wherein the hexavalent chromium is introduced as compounds selected from the group consisting of chromic anhydride, chromates of ammonium, beryllium, potassium, cadmium, lithium, magnesium, sodium, zinc, bichromates of ammonium, beryllium, potassium, cadmium, lithium, magnesium, sodium, zinc, mixtures of said chromates, mixtures of said bichromates, mixtures of said chromates and bichromates, and mixtures of chromic anhydride

and chromates, mixtures of chromic anhydride and bichromates, mixtures of chromic anhydride, chromates and bichromates,

15 5. A composition for color passivation of zinc and cadmium as claimed in claim 1, wherein the nitrate is introduced as compounds selected from the group consisting of nitrates of ammonium, beryllium, potassium, cadmium, lithium, magnesium, sodium, and zinc.

20 6. A composition for the color passivation of zinc and cadmium as claimed in claim 1, wherein the sulphate is introduced as compounds selected from the group consisting of sulphates of ammonium, beryllium, potassium, cadmium, lithium, magnesium, sodium, zinc, and bisulphates of ammonium potassium, lithium, and sodium.

25 7. A composition for the color passivation of zinc and cadmium as claimed in claim 1, wherein the boron is introduced as compounds selected from the group consisting of boric acid, magnesium orthoborate, and polyborates of ammonium, beryllium, potassium, lithium, magnesium, and sodium.

30 8. A composition for the color passivation of zinc and cadmium as claimed in claim 1, wherein the amino acid has the general formula:



35 40 whereof  $R_1$  and  $R_2$  stand for  $-H$ ,  $-\text{CH}_3$ ,  $-\text{C}_2\text{H}_5$ ,  $-\text{C}_3\text{H}_7$ ,  $-\text{C}_4\text{H}_9$ ,  $-\text{C}_6\text{H}_5$ ,  $-\text{CH}_2\text{OOH}$ ,  $-\text{CH}_2\text{OOH}$ ,  $-\text{CH}_2\text{CH}_2\text{COOH}$ ,  $-\text{CH}_2\text{CH}_2\text{OH}$ ,  $-\text{CH}_2\text{CH}_2\text{CN}$ ,  $-\text{CH}_2\text{CH}_2\text{COCH}_3$ ,  $-\text{CH}_2\text{CH}_2\text{COC}_2\text{H}_5$ ,  $-\text{CH}_2\text{CH}_2\text{COC}_3\text{H}_7$ ,  $-\text{CH}_2\text{CH}_2\text{COC}_6\text{H}_5$ ;  $R_3$  and  $R_4$ , for  $-H$ ,  $-\text{CH}_3$ ,  $-\text{C}_3\text{H}_5$ ,  $-\text{C}_3\text{H}_7$ ,  $-\text{C}_4\text{H}_9$ ,  $-\text{C}_5\text{H}_{11}$ ,  $-\text{C}_6\text{H}_{13}$ ,  $-\text{C}_7\text{H}_{15}$ ,  $-\text{C}_8\text{H}_{17}$ ,  $-\text{CH}_2\text{COOH}$ ,  $-\text{CH}_2\text{CH}_2\text{COOH}$ ,  $-(\text{CH}_2)_k\text{NH}_2$ ,  $-(\text{CH}_2)_k$



55 50  $\text{C}_6\text{H}_5$ ,  $K=1-4$  and  $n=1-5$ .

45 55 9. A composition for the color passivation of zinc and cadmium as claimed in claim 1, wherein the content of its ingredients in the aqueous solution thereof being (in g/l):

|                                                       |          |
|-------------------------------------------------------|----------|
| hexavalent chromium compound (calculated as chromium) | 1.7-70.0 |
| nitrate compound (calculated as $\text{NO}_3^-$ )     | 1.0-45.0 |
| sulphate compound (calculated as $\text{SO}_4^{2-}$ ) | 1.0-25.0 |
| boron compound (calculated as boron)                  | 0.5-10.0 |
| amino acid                                            | 0.05-6.0 |

60 and the solution pH = 1.1-2.8.

65 10. A composition for the color passivation of zinc and cadmium as claimed in claim 9, wherein the con-

tent of its ingredients in the aqueous solution thereof being (in g/l):

|                                                       |           |   |
|-------------------------------------------------------|-----------|---|
| hexavalent chromium compound (calculated as chromium) | 11.0-21.0 | 5 |
| nitrate compound (calculated as $\text{NO}_3^-$ )     | 2.4-6.0   |   |
| sulphate compound (calculated as $\text{SO}_4^{2-}$ ) | 2.2-7.0   |   |
| boron compound (calculated as boron)                  | 1.1-4.3   |   |
| amino acid                                            | 0.05-0.1  |   |

solution pH = 1.6-2.3.

11. A composition for the color passivation of zinc and cadmium as claimed in claim 9, wherein the content of its ingredients in the aqueous solution thereof are (in g/l):

|                                                       |           |
|-------------------------------------------------------|-----------|
| hexavalent chromium compound (calculated as chromium) | 11.0-21.0 |
| nitrate compound (calculated as $\text{NO}_3^-$ )     | 2.4-6.0   |
| sulphate compound (calculated as $\text{SO}_4^{2-}$ ) | 2.2-7.0   |
| boron compound (calculated as boron)                  | 1.1-4.0   |
| amino acid                                            | 0.5-4.0   |

solution pH = 1.6-2.3.

12. A method for the color passivation of zinc and cadmium by comprising dipping them into an aqueous solution of the composition as claimed in claim 9 for a period of 3 to 90 seconds at a temperature of from 15° to 35°C.

\* \* \* \* \*

15

20

25

30

35

40

45

50

55

60

65